# EUROPEAN PATENT SPECIFICATION

(11) **EP 1 752 563 B1**
(45) Date of publication and mention of the grant of the patent: **05.10.2016**
(21) Application number: 06254217.0
(22) Date of filing: 10.08.2006
(51) Int. Cl.: C25F 5/00

(54) **Masking techniques for electrochemical stripping**
Maskierungstechnik bei elektrochemischem Strippen
Technique de masquage pour l'enlèvement électrochimique des revêtements

(30) Priority: 12.08.2005 US 203055
(43) Date of publication of application: 14.02.2007
(62) Divisional of application: 12159393.3
(73) Proprietor: United Technologies Corporation, Hartford, CT 06101 (US)
(72) Inventor: Riewe, Curtis Heath, Manchester, CT 06040 (US); Griffith, Brian J., Vernon, CT 06066 (US)
(74) Representative: Leckey, David Herbert

(56) References cited:
- KR-A- 20010 065 374
- US-A- 3 855 083
- US-A- 4 401 523
- US-A1- 2003 168 350
- US-A1- 2004 134 066

## Description

### BACKGROUND OF THE INVENTION

The present invention relates to an improved technique for masking airfoils during electrochemical stripping operations.

It has been found that wall thinning of an airfoil portion of a turbine engine component will occur as a result of removing a coating applied to the airfoil portion and/or a diffusion layer formed on the airfoil portion using electrochemical stripping techniques. Wall thinning is highly undesirable because it leads to bending.

Prior art documents that relate to electroplating include KR-A-2001/0065374, which describes an electroplating method for preventing excessive plating of an edge, US-A-4401523, which describes an apparatus and method for plating metallic strip, and US-A-2004/0134066, which describes methods and apparatus for manufacturing turbine engine components.

US-A-2003/0168350 describes a stripping process having the features of the preamble of claim 1.

Thus, it is deemed desirable to mask the trailing edges of airfoils used in turbine engine components, such as vanes and blades, to prevent wall thinning and cooling hole closure caused by bending a thin wall. Many of the techniques employed today use non-conductive trailing edge maskants to prevent this from occurring. Typically, barrier types of maskants, such as plater's tape, lacquer, and UV-curable materials, have been used in the stripping processes.

Some of the maskants which have been used have caused trenching of the airfoil portion under the masked area. The trench is caused by crevice corrosion and is an unacceptable condition. It is speculated that the trench is formed as a result of a crevice being formed under the maskant as the coating and/or diffusion layer are removed. After the crevice is formed, crevice corrosion begins and propagates, causing the formation of the trench.

There is a need for improved maskant materials, particularly those which help avoid trenching.

### SUMMARY OF THE INVENTION

The invention provides a method for removing a coating from an airfoil portion of a turbine engine component as claimed in claim 1. The edge can be a trailing edge of said airfoil portion.

### BRIEF DESCRIPTION OF THE DRAWINGS

Fig. 1 illustrates a trailing edge portion of a turbine engine component having windows;
Fig. 2 illustrates the application of a UV curable maskant to the trailing edge;
Fig. 3 is a schematic representation of a first embodiment of a maskant;
Fig. 4 is a schematic representation of a clip; and
Figs. 5 - 7 illustrate an alternative embodiment of a clip.

### DETAILED DESCRIPTION OF THE PREFERRED EMBODIMENT(S)

As discussed above, the present disclosure relates to a masking technique for use in a method for electrochemically stripping coatings and/or diffusion layers from airfoil portions of turbine engine components, such as turbine blades, vanes, seals and shrouds. In one embodiment, the maskant for the trailing edge of the airfoil portion comprises a layer of a UV curable maskant material and a clip placed over the UV curable maskant formed from an electrically conductive material. Preferably, the electrically conductive material is formed from a titanium based material. Titanium is a preferred material because it will not corrode in many of the baths used in electrochemical stripping techniques. Root portions of the turbine engine component may be masked by dipping the root portions into a thin paint or by applying a lacquer in order to prevent any slight etching or pitting. In another embodiment, the maskant solely comprises a clip placed over the airfoil trailing edge.

The masking technique of the present invention may be used in conjunction with any suitable electrochemical stripping technique known in the art.

Referring now to Fig. 1, a trailing edge portion 22 of an airfoil portion 4 is shown. The trailing edge portion 22 has a plurality of windows or openings 6 which need to be protected during the electrochemical stripping technique.

In accordance with an embodiment of the present invention, as shown in Fig. 2, a UV curable maskant 2, such as DYMAX UV MASKANT-29605, is placed on the trailing edge portion 22 of an airfoil portion 4 of a turbine engine component, such as a turbine blade or vane. The UV curable maskant 2 preferably covers any trailing edge windows 6. The coverage of the UV curable maskant is dependent on part configuration. It is important that the UV maskant be applied so that a clip 30 may be placed on top of it. Typically, the UV curable maskant will cover up to 0.2 inches (5.1 mm) from the trailing edge on the concave side. After being applied, the maskant 2 is cured in a UV oven and checked for completeness of coverage. Thereafter, an electrically conductive member 10, preferably formed from a titanium based material, is placed over the maskant 2 on the trailing edge portion 22 of the airfoil 4. It has been found that the use of an electrically conductive member 10, such as one formed from a titanium based material, helps prevent the masked area from being completely stripped and helps prevent crevice corrosion, and thus trenching, from occurring. This is because the electrically conductive member 10 acts as a current thief or current shield which prevents the coating material and/or diffusion layer beneath the maskant from being removed.

Using the masking technique of the present invention, it is possible to obtain a coating remaining on the airfoil portion trailing edge of the turbine engine component which has a smooth transition between the fully stripped base alloy forming the turbine engine component and the fully protected coating. A smooth transition is desirable because it significantly reduces or eliminates any subsequent blending of the coating needed to remove any sharp corner.

As shown in FIG. 3, the electrically conductive member 10 may comprise two bars 12 and 14 of a titanium based material bolted together via a bolt 16 and placed over opposed surfaces 18 and 20 of the trailing edge 22 having the UV curable maskant 2 applied thereto. Alternatively, as shown in FIG. 4, the member 10 may comprise a titanium foil member or clip 30 held onto the trailing edge 22 of the airfoil portion of the turbine engine component by one or more securing elements 32 or by friction. The securing elements 32 may be formed from any conductive material that does not corrode. A preferred material for each element 32 is titanium. When a titanium clip 30 is used, the member 30 may have a thickness in the range of from 0.020 to 0.030 inches (0.51 - 0.76 mm).

FIGS. 5 - 7 illustrate a preferred configuration for the clip 30 which can be used without any UV maskant. As can be seen, the clip 30 has a folded over piece 50 of an insulating material such as silicon rubber. The piece 50 conforms to the part and continues to seal the part as the coating is stripped away under it. This reduces the tendency to form trenches. On top of the insulating material piece are layers 52 and 54 formed from an electrically conductive material such as a titanium based material. The two layers 52 and 54 are joined to each other by a hinge structure 56. The hinge structure 56 allows the layers 52 and 54 to move relative to each other. When the clip 30 is placed over the trailing edge 22 of the airfoil portion of the turbine engine component, one or more variable positionable C-shaped securing member 58 may be placed over the layers 52 and 54. If desired, the securing members 58 may be formed from a plastic material. Still further, if desired, a UV curable maskant may be used under the clip 30.

Prior to, or subsequent to, applying the electrically conductive member 10 or clip 30, root portions of the turbine engine component may be masked to prevent any slight etching or pitting. Masking of the root portions may be achieved by dipping them into a thin paint, such as DYKEM layout ink fluid, or by hand applying a maskant, such as a suitable lacquer. Preferably, two coats of the root portion masking material should be applied. After application of the root portion masking material, the turbine engine component may be subjected to a drying treatment which depends upon the nature of the root portion maskant.

As previously mentioned, the use of an electrically conductive member 10 or clip 30, particularly one formed from a titanium based material, helps prevent trenching. It also provides a smoother transition between the coating on the trailing edge portion of the turbine engine component and the underlying substrate.

### EXAMPLE

Two high pressure turbine blades were stripped in a 4.7 vol.% hydrochloric acid solution at a temperature of approximately 20°C. The stripping potential set point was 0.08v with respect to an Ag/AgCl reference electrode. The turbine blades were stripped for 2 hours, water pressure sprayed, tripped for an additional two hours, burnt out, grit blasted, and heat tinted. All of the blades were masked at the root and the tip with Dymax X-391-17A. One of the blades had a U-channel mask in accordance with the present invention applied to the trailing edge. The other of the blades had a hinged clip in accordance with the present invention applied to the trailing edge. The test showed an absence of crevice corrosion at the trailing edge.

While the masking technique of the present invention preferably applies a UV curable material over the trailing edge portion, for removing certain coatings from some turbine engine components, the UV curable material may be omitted.

While the UV curable material may be applied to both sides of the trailing edge portion of the turbine engine component, it may also be applied to just one side such as the concave side.

After the trailing edge portions of the root portion have been masked, the turbine engine component is immersed in an acidic bath. The bath may be any suitable stripping bath known in the art. After immersion, the coating on the turbine engine component may be stripped using any suitable electromechanical stripping technique known in the art. The particular electrochemical stripping technique does not form part of the present invention.

While the present invention has been described with the maskant placed about a trailing edge of an airfoil portion of a turbine engine component, the maskant could also be applied to a leading edge or a tip of the airfoil portion and/or to a platform portion of the component.

## Claims

1. A method for removing a coating from an airfoil portion (4) of a turbine engine component **characterised by** comprising the steps of:
placing a maskant (10; 30) formed from an electrically conductive material on opposed sides of an edge (22) of said airfoil portion (4);
immersing said turbine engine component with said maskant into a bath; and
electrochemically stripping a coating from unmasked portions of said turbine engine component.

2. A method according to claim 1, further comprising applying a UV curable material (2) to at least one side of said edge (22) prior to said maskant placing step and placing said maskant (10; 30) over said UV curable material (2).

3. A method according to claim 1 or 2, wherein said maskant placing step comprises placing a maskant (10; 30) formed from a titanium based material on opposed sides of said edge (22).

4. A method according to claim 1 or 2, wherein said maskant placing step comprises placing two bars (12, 14) formed from a titanium based material on opposed sides of said edge (22) and bolting said bars (12, 14) together.

5. A method according to claim 1 or 2, wherein said maskant placing step comprises placing a clip (30) formed from a titanium based material on opposed sides of said edge (22) and securing said clip to said edge (22).

6. A method according to claim 1 or 2, wherein said maskant placing step comprises placing a clip having a layer of insulating material (50) and a pair of plates (52, 54) each formed from a titanium based material on opposed sides of the edge (22) and securing said clip (30) to said edge.

7. A method according to any of claims 1 to 6, further comprising placing a maskant on root portions of said turbine engine component.

8. A method according to claim 7, wherein said root portion masking step comprises applying a masking paint or a lacquer to said root portions.

9. A method according to any of claims 1 to 8, wherein said edge (22) is a trailing edge of said airfoil portion (4).

## Patentansprüche

1. Verfahren zum Entfernen einer Beschichtung von einem Schaufelblattabschnitt (4) eines Turbinenmotorbauteils, **dadurch gekennzeichnet, dass** es folgende Schritte umfasst:
Anordnen eines Maskierungsmittels (10; 30), das aus einem elektrisch leitfähigen Material gebildet ist, auf gegenüberliegenden Seiten einer Kante (22) des Schaufelblattabschnitts (4);
Eintauchen des Turbinenmotorbauteils mit dem Maskierungsmittel in ein Bad; und
elektrochemisches Strippen einer Beschichtung von unmaskierten Abschnitten des Turbinenmotorbauteils.

2. Verfahren nach Anspruch 1, ferner umfassend Aufbringen eines UV-härtbaren Materials (2) auf wenigstens eine Seite der Kante (22) vor dem Schritt des Anordnens des Maskierungsmittels und Anordnen des Maskierungsmittels (10; 30) über dem UV-härtbaren Material (2).

3. Verfahren nach Anspruch 1 oder 2, wobei der Schritt des Anordnens des Maskierungsmittels das Anordnen eines Maskierungsmittels (10; 30), das aus einem Material auf Titanbasis gebildet ist, auf gegenüberliegenden Seiten der Kante (22) umfasst.

4. Verfahren nach Anspruch 1 oder 2, wobei der Schritt des Anordnens des Maskierungsmittels das Anordnen von zwei Leisten (12, 14), die aus einem Material auf Titanbasis gebildet sind, auf gegenüberliegenden Seiten der Kante (22) und das Verschrauben der Leisten (12, 14) miteinander umfasst.

5. Verfahren nach Anspruch 1 oder 2, wobei der Schritt des Anordnens des Maskierungsmittels das Anordnen einer Klemme (30), die aus einem Material auf Titanbasis gebildet ist, auf gegenüberliegenden Seiten der Kante (22) und das Befestigen der Klemme an der Kante (22) umfasst.

6. Verfahren nach Anspruch 1 oder 2, wobei der Schritt des Anordnens des Maskierungsmittels das Anordnen einer Klemme mit einer Schicht Isoliermaterial (50) und einem Paar Platten (52, 54), die jeweils aus einem Material auf Titanbasis gebildet sind, auf gegenüberliegenden Seiten der Kante (22) und das Befestigen der Klemme an der Kante (30) umfasst.

7. Verfahren nach einem der Ansprüche 1 bis 6, ferner umfassend Anordnen eines Maskierungsmittels auf Fußabschnitten des Turbinenmotorbauteils.

8. Verfahren nach Anspruch 7, wobei der Schritt des Maskierens des Fußabschnitts das Aufbringen eines Maskierungsanstrichs oder eines Lacks auf die Fußabschnitte umfasst.

9. Verfahren nach einem der Ansprüche 1 bis 8, wobei die Kante (22) eine Hinterkante des Schaufelblattabschnitts (4) ist.

## Revendications

1. Procédé d'élimination d'un revêtement sur une partie de profilé (4) d'un composant de moteur de turbine **caractérisé par** le fait de comprendre les étapes suivantes :
placement d'un masquant (10 ; 30) formé d'un matériau électroconducteur sur les côtés opposés d'un bord (22) de ladite partie de profilé (4) ;
immersion dudit composant de moteur de turbine avec ledit masquant dans un bain ; et
décapage électrochimique d'un revêtement sur des parties non masquées dudit composant de moteur de turbine.

2. Procédé selon la revendication 1, comprenant en outre l'application d'un matériau durcissable aux UV (2) sur au moins un côté dudit bord (22) avant ladite étape de placement de marquant et le placement dudit masquant (10 ; 30) sur ledit matériau durcissable aux UV (2).

3. Procédé selon la revendication 1 ou 2, dans lequel ladite étape de placement de masquant comprend un masquant (10 ; 30) formé d'un matériau à base de titane sur les côtés opposés dudit bord (22).

4. Procédé selon la revendication 1 ou 2, dans lequel ladite étape de placement de masquant comprend le placement de deux barres (12, 14) formées d'un matériau à base de titane sur les côtés opposés dudit bord (22) et le boulonnage desdites barres (12, 14) ensemble.

5. Procédé selon la revendication 1 ou 2, dans lequel ladite étape de placement de masquant comprend le placement d'une pince (30) formée d'un matériau à base de titane sur les côtés opposés dudit bord (22) et la fixation de ladite pince audit bord (22).

6. Procédé selon la revendication 1 ou 2, dans lequel ladite étape de placement de masquant comprend le placement d'une pince comportant une couche de matériau isolant (50) et une paire de plaques (52, 54), chacune étant formée d'un matériau à base de titane, sur les côtés opposés du bord (22) et la fixation de ladite pince (30) audit bord.

7. Procédé selon l'une quelconque des revendications 1 à 6, comprenant en outre le placement d'un masquant sur des parties d'embase dudit composant de moteur de turbine.

8. Procédé selon la revendication 7, dans lequel ladite étape de masquage de partie d'embase comprend l'application d'une peinture ou d'un vernis de masquage destiné aux dites parties d'embase.

9. Procédé selon l'une quelconque des revendications 1 à 8, dans lequel ledit bord (22) est un bord de fuite de ladite partie de profilé (4).
